

## UNITED STATES PATENT OFFICE

CHARLES L. MANTELL, OF BROOKLYN, NEW YORK, ASSIGNOR TO DUDZEELE CORPORATION OF AMERICA, OF NEW YORK, N. Y., A CORPORATION OF DELAWARE

## ART OF REMOVING LEAD FROM FERROUS ARTICLES

No Drawing. Application filed March 29, 1929, Serial No. 351,131. Renewed March 14, 1932.

My invention relates to the art of removing coatings of lead or lead alloys from tubes or other ferrous articles, such as tere plate, scrap, rods, wire, etc.

5 Broadly, the invention consists in removing the lead coating by subjecting the article (as by immersion) to a solution containing appreciable amounts of chlorides and hydrogen ions resulting from the use of a non-10 oxidizing mineral acid with a small amount of a catalytic material such as nickel, salts; for example, chloride or sulphate of nickel.

Lead is one of the best known metals employed as a material of construction for corrosion resistance. Its use in the manufacture of sulphuric acid and in the chemical industries is well known. It is quite resistant to many forms of chemical attack. The invention aims to remove lead or lead alloys 15 from articles by subjecting them to a solution which attacks and removes or enables the removal of the lead without considerable or objectionable attack upon the ferrous article. The employment of a catalyst such as above referred to materially expedites or speeds up the reaction upon the lead coating and thus by reducing the time of subjection of the article to the deleading bath, reduces the corrosion effect upon the main body of the 20 article.

In carrying out the process in one approved way, the tubes or other articles to be deleaded are first cleaned in an alkaline solution, such as sodium hydroxide, at a temperature preferably near the boiling point; or heated aqueous solutions of so-called commercial cleaners may be employed, or alkali solutions with emulsifying agents such as sulphonated oils, and various detergents (as sodium carbonate, 25 phosphates, etc.).

After cleaning, the articles are immersed in the deleading solution in the same general manner or method which is employed in pickling rolled or drawn steel articles.

45 A preferred deleading solution, as generally described, comprises appreciable amounts of chlorides and hydrogen ions resulting from the use of a non-oxidizing mineral acid with a small amount of a catalyst, such as 50 nickel salts, or equivalent.

As a specific example of one approved solution, the following ingredients and proportions are stated:

Sodium chloride (common salt) in concentrations from about 15% of weight up to 55 saturation, acidified by approximately 5% sulphuric acid, and as a catalyst, a nickel salt, such as chloride or sulphate or nickel, in concentrations from as low as one one-thousandth of 1% to as high as five-tenths of 1%. The 60 sulphuric acid reacts with part of the sodium chloride to form hydrochloric acid and sodium acid sulphate. The bath contains a greater quantity of sodium chloride than is chemically equivalent to the amount of sulphuric 65 acid specified. A commercially satisfactory result is obtained with the catalyst in the range of one one-thousandth of 1% to one-tenth of 1%. Hydrochloric acid may be substituted for the sulphuric acid, the sulphuric 70 being preferred in commercial work because it is a cheaper reagent.

In plant operation it is desired that the solution shall work upon and remove the lead without marked effect on the ferrous metal 75 or alloy composing the main bulk of the fabricated article. The addition of nickel salts to the bath has been found markedly to speed up the reaction, and thus to reduce attack upon the ferrous body. The bath is desirably 80 maintained at a temperature from 180° F. up to the boiling point of the solution.

After removal from the deleading bath the articles are washed, preferably in hot water, to dissolve and wash off any lead chloride or 85 lead salts still adhering.

The time required for deleading is a function of the size of the article, the thickness of the coating, and the surface finish desired.

Soluble platinum salts may be used in low 90 concentrations in place of nickel salts, but are usually unavailable for this purpose because of the higher cost. Accordingly, whenever I refer in the claims to nickel salts as 95 the catalyst, I mean any material which is substantially the equivalent of nickel salts in the sense that it will bring about to a practical extent the results herein attributed to the presence of nickel salts. It is believed 100

that the catalytic action of the nickel salt is as follows:

The nickel ions are precipitated as nickel atoms on the surface of the lead to form a nickel lead electrolytic couple, as the result of 5 which the attack on the lead and its resultant solution is accelerated.

The present invention is an improvement upon that disclosed in my prior application, Serial No. 325,643, filed December 12, 1928, 10 and consists largely in the addition to certain typical deleading solutions therein disclosed, of a catalyst of the character and for the purposes above described.

I claim:

15 1. A deleading solution containing appreciable amounts of chlorides and hydrogen ions resulting from the use of a non-oxidizing mineral acid, with a small proportion of a nickel salt as a catalyst.

20 2. A deleading solution containing sodium chloride in concentrations from approximately 15% by weight up to saturation, and approximately 5% non-oxidizing mineral acid, and a nickel salt as a catalyst in concentrations from approximately 1000th of 1% to approximately  $\frac{1}{10}$  of 1%.

25 3. A deleading solution containing sodium chloride concentrations from approximately 15% by weight up to saturation, and approximately 5% sulphuric acid, and a nickel salt as a catalyst in concentrations from approximately 1000th of 1% to approximately  $\frac{1}{10}$  of 1%.

30 4. A deleading solution containing sodium chloride in concentrations from approximately 15% by weight up to saturation, and approximately 5% non-oxidizing mineral acid, and a nickel salt in small percentage as a catalyst.

35 5. A deleading solution containing sodium chloride concentrations from approximately 15% by weight up to saturation, and approximately 5% sulphuric acid, and a nickel salt in relatively low concentration as a catalyst.

40 6. A deleading process including, as a characteristic operation, subjecting a lead-coated ferrous article to a solution comprising appreciable amounts of chlorides and hydrogen ions resulting from the use of a non-oxidizing mineral acid, with a small proportion of a nickel salt as a catalyst.

45 7. A deleading process including as a characteristic operation subjecting a lead-coated ferrous article to a solution comprising sodium chloride in concentrations from approximately 15% by weight up to saturation, and approximately 5% non-oxidizing mineral acid, and a nickel salt as a catalyst in concentrations from approximately 1000th of 1% to approximately  $\frac{1}{10}$  of 1%.

50 8. A deleading process including, as a characteristic operation, subjecting a lead-coated ferrous article to a solution comprising appreciable amounts of chlorides and

hydrogen ions resulting from the use of a non-oxidizing mineral acid, with a small proportion of a nickel salt as a catalyst, the bath being maintained at a temperature near boiling.

70 9. A deleading process including, as a characteristic operation, subjecting a lead-coated ferrous article to a solution comprising appreciable amounts of chlorides and hydrogen ions resulting from the use of a non-oxidizing mineral acid, with a small proportion of a nickel salt as a catalyst, the bath being maintained at a temperature from approximately 180° F. to boiling.

75 10. A deleading process including as a characteristic operation subjecting a lead-coated ferrous article to a solution comprising appreciable amounts of chlorides and hydrogen ions resulting from the use of a non-oxidizing mineral acid, with a small proportion of a nickel salt as a catalyst, the bath being maintained at a temperature near boiling.

80 11. The described process, including as characteristic features, cleaning lead-coated ferrous articles in an alkaline solution, subjecting them to a deleading bath of character described in claim 1, and washing the articles to remove remaining lead and deleading solution.

85 12. The described process including as characteristic features, cleaning lead-coated ferrous articles in an alkaline solution, subjecting them to a deleading bath of character described in claim 2, and washing the articles to remove remaining lead and deleading solution.

90 13. A deleading solution containing appreciable amounts of chlorides and hydrogen ions, with nickel salt as a catalyst.

95 In testimony whereof I affix my signature.

CHARLES L. MANTELL.

110

115

120

125

130